

March 11, 1924.

1,486,804

C. H. RUDER ET AL

APPARATUS FOR SILVERING

Original Filed Aug. 19, 1922

Fig. 1.



Fig. 2.



Inventor.  
Charles H. Ruder  
and  
George M. D. Shadwick  
by Miller, Henry & Boykin  
Attorneys.

## UNITED STATES PATENT OFFICE.

CHARLES H. RUDER AND GEORGE M. D. SHADWICK, OF SAN FRANCISCO, CALIFORNIA.

## APPARATUS FOR SILVERING.

Application filed August 19, 1922, Serial No. 583,000. Renewed January 14, 1924.

*To all whom it may concern:*

Be it known that we, CHARLES H. RUDER and GEORGE M. D. SHADWICK, citizens of the United States, and residents of the city and county of San Francisco, State of California, have invented a new and useful Apparatus for Silvering, of which the following is a specification.

Our invention has for its object the depositing on a portion of the surface of an incandescent lamp bulb a metallic reflecting surface, which will be hard and durable and free from injury such as heat and exposure when the lamp is in service.

Other objects will appear from the specifications which follow.

These objects we accomplish by mounting the lamp with the filament portion downward with respect to the silvering solution during the period that the deposit is being made upon the lamp surface. The silvering we accomplish by applying a small quantity of solution adjacent the glass surface of the lamp where the deposit is to be made, said solution being contained within a cup of hard rubber or other inert material formed of suitable shape and having a soft gasket in the lower portion into which the lamp is fitted, thereby sealing the bottom of the cup against leakage of the solution. The solution is then poured around the lamp and the filament energized by an electric current whereby the glass surface of the lamp and the adjacent solution is heated.

We attach special importance to the position of the filament being downward with respect to the solution, thereby maintaining the solution during the depositing period adjacent to the hottest portion of the lamp and securing an advantageous circulation of the solution which results in a maximum amount of closely adhering metallic deposit on the glass surface instead of on the surface of the cup or container.

By referring to the accompanying drawing our invention will be made clear.

Fig. 1 illustrates a lamp in position in the cup or container which latter is shown in cross section and as positioned during the period of treatment and also shows the electrical connections from the swinging arm which we employ for centering and energizing the lamp.

Fig. 2 is a view of the apparatus of Fig. 1 and at right angles thereto.

Fig. 3 is one of our completed lamps showing the manner in which light is distributed upward by the frosted surface between the lower limit of the silvered surface 19 and the equator 21.

Throughout the figures similar numerals refer to identical parts.

The lamp which is to be silvered is indicated by the numeral 1. Its spherical portion is pressed into place against the soft gasket 2 forming the bottom portion of the cup 3. The silvering solution 4 is then poured around the lamp to the desired depth 5 and the arm 6 swung from its dotted to the full line position, and the electric circuit is completed through the spring member 7 and the latch member 8, these forming the two terminals from any conventional source of electrical energy furnished through the double cord 9 and socket 10. The cup 3 is carried on any suitable support 11 which may be arranged to receive a plurality of cups, for each of which there is a swinging arm 6. The lamp bulb projects through an opening 12 in the support 11 and its filament 13 projects downward to or below the zone of silvering 14.

At 15 and 16 are indicated conventional hinges and wall support.

On account of the position of the filament below the silverizing zone, the greatest amount of heat is distributed from the filament against the glass wall to be silvered, thus securing a more active solution from which the metallic deposit is made. This we have found secures a more perfect coherence between the deposit and the glass surface and secures a thicker and firmer deposit in less time and with greater economy in the reagents used than has been heretofore attained.

Before placing the lamp in the cup 3 the glass surface is to be chemically cleaned and we prefer to employ for this a solution consisting of one pound bichromate of potash in 300 c. c. of water and 1500 c. c. of sulphuric acid into which the lamp is to be immersed about 10 seconds, then washed in running water and finally in distilled water.

The process includes the employment of a silvering solution composed substantially of  $7\frac{1}{2}$  grams nitrate of silver; 5 grams sulphate of copper; 2 grams sulphate of nickel, which are to be dissolved separately and then mixed. A sufficient quantity of am-

monia is then added to turn the solution a deep blue, after which a saturated solution of tartaric acid is added until the solution takes on an opalescent tint, after which distilled water is added to make 1000 c. c. of solution.

After the lamp has been placed in the position shown in Figs. 1 and 2 and solution above described added up to the desired line 10 5 the filament 13 is energized by engaging the contacts 7 and 8 with the lamp base by swinging the arm 6 downward on the hinge 15.

The hottest portion of the lamp will now 15 be in the zone 5 to 14. The solution is heated thereby and the circulation within the said solution, due to the hot glass surface, takes place in the direction of the arrows 20 17 and 18 causing a metallic deposit of silver, copper and nickel on the glass surface, which will be of the requisite thickness in about one hour.

The arm 6 is then swung up and the lamp 25 removed and while still moist is to be dipped in a solution of 10% mercuric cyanide, after which the lamp is rinsed in clear water and the deposit allowed to dry hard.

The coating may now be trimmed as to the 30 line 19 to remove the feather edge and if desired the lamp may be frosted over the unsilvered portion of its spherical surface 20 up to the line 19. We prefer to carry this frosting substantially 10 degrees above the equatorial portion 21 of the bulb so that 35 when the lamp is in a depending position in a fixture the diffused illumination secured from the surface above the equatorial portion and up to the line 19 diffuses upward

a sufficient illumination to reduce shadows on the fixture or ceiling 23 to a minimum. 40

This result is best shown in Fig. 3 where in the equatorial line of the spherical surface is shown at 21 above which the frosted surface extending to 19 forms a source of illumination indicated by the rays as 22, 45 which falling upon the ceiling 23 reduces shadows thereon to a minimum.

We claim:

1. Apparatus for silvering an incandescent lamp consisting of a cup provided with an open bottom having a soft gasket adapted to snugly hold the equatorial portion of an incandescent lamp and leaving a portion of the glass surface exposed within the cup and above the lamp filament. 50

2. Apparatus for silvering an incandescent lamp consisting of a cup provided with an open bottom having a soft gasket adapted to snugly hold the equatorial portion of an incandescent lamp and leaving a portion 30 of the glass surface exposed within the cup and above the lamp filament, and movable contacts adapted to engage and energize the lamp.

3. Apparatus for silvering an incandescent lamp consisting of a cup provided with an open bottom having a soft gasket adapted to snugly hold the equatorial portion of an incandescent lamp and leaving a portion 40 of the glass surface exposed within the cup and above the lamp filament, and movable contacts adapted to engage and energize the lamp, said contacts carried on a swinging arm. 55

CHARLES H. RUDER.  
GEORGE M. D. SHADWICK